

Dec. 4, 1956

J. D. C. WILSON II

2,772,995

LEATHER REPLACEMENT COMPOSITIONS AND PROCESS

Filed May 7, 1954

3 Sheets-Sheet 1

FIG. 1



JOSEPH DURANT COOPER WILSON, II

BY

*A. Ralph Snyder*

ATTORNEY

Dec. 4, 1956

J. D. C. WILSON II

2,772,995

LEATHER REPLACEMENT COMPOSITIONS AND PROCESS

Filed May 7, 1954

3 Sheets-Sheet 2

## FIG. 2



INVENTOR

JOSEPH DURANT COOPER WILSON, II

BY

*A. Ralph Snyder*

ATTORNEY

Dec. 4, 1956

J. D. C. WILSON II

2,772,995

LEATHER REPLACEMENT COMPOSITIONS AND PROCESS

Filed May 7, 1954

3 Sheets-Sheet 3

FIG. 3



INVENTOR

JOSEPH DURANT COOPER WILSON, II

BY

*J. D. C. Wilson*

ATTORNEY

2,772,995

## LEATHER REPLACEMENT COMPOSITIONS AND PROCESS

Joseph Durant Cooper Wilson II, New Castle, Del., assignor to E. I. du Pont de Nemours and Company, Wilmington, Del., a corporation of Delaware

Application May 7, 1954, Serial No. 428,356

12 Claims. (Cl. 154—124)

This invention relates to leather replacement compositions and, more particularly, to leather replacement sheets having outstanding resistance to fuzzing upon being subjected to scuffing or abrasion.

Patents relating to methods and techniques of preparing leather replacement compositions have been granted to inventors as far back as 1850; and even before that time, a great number of attempts had been made to devise a simple and rapid technique of producing leather replacement compositions. In most of the early art, pyroxylin was used to coat or impregnate various types of fibrous base materials to prepare leather substitutes. As time went on, pyroxylin/oil/pigment compositions were widely used as coating or impregnating compositions for various woven or non-woven fibrous base materials. In the early stages of the synthetic leather industry, the main objective was to simulate the general appearance of leather.

In today's markets, coated fabrics, particularly the vinyl-coated fabrics, are outstanding as leather substitutes in such applications as handbags, bookbindings, brief cases, card table covers, luggage, etc. In such applications, the coated fabrics are satisfactory because the general appearance of leather is simulated; and the coated fabrics possess some of the desirable properties of leather. However, as compared to genuine leather, the coated fabrics lack good tear strength, softness and the ability to "breathe" or transpire water vapor and air; and although the coated fabrics are used in such applications as chair coverings, much is left to be desired, especially with respect to water vapor and air permeability. Up to the present time, leather replacement compositions have made little or no inroads into the boots, shoes, and gloves markets, mainly because of their inability to breathe in addition to lack of good tear strength and softness. As used hereinafter, the term "breathe" means transpire water vapor and air.

In general, the use of leather replacement compositions in boots, shoes, gloves, etc., is mainly dependent upon its ability to breathe, usually expressed in terms of water vapor permeability or "leather permeability." Physical tests on the water vapor permeability of leather indicate that leather transpires water vapor about two-thirds as readily as free air. In general terms, shoe upper leather samples having a thickness of 0.016"-0.104" have a leather permeability within the range of 2,000-18,000 grams/100 sq. meters/hour when tested according to the method of Kanagy and Vickers Journal of American Leather Chemists Association 45, 211-242 (April 1950) in an atmosphere of 23° C. and 90% relative humidity. Hereinafter, the ability of leather replacement compositions to transpire water vapor will be expressed in terms of leather permeability in the units of grams/100 sq. meters/hour. Based upon comfort tests, the minimum tolerable leather permeability for shoe upper leather is about 2,000 grams/100 sq. meters/hour. Preferably for shoe upper leather, the permeability value should be

4,000-20,000 when tested at 23° C. and not greater than 90% relative humidity.

Recently, various techniques and processes have been developed for preparing leather replacement compositions which not only have the appearance of leather, but are also capable of breathing. Comparisons of the leather permeability of these leather replacement compositions compared with genuine leather have shown that the leather permeability of these compositions in many cases is superior to that of shoe uppers fabricated from genuine leather. Furthermore, the flexibility of these recently developed techniques provides for tailoring the compositions for particular end uses, that is, produces a product having the desired water vapor permeability, tear strength, softness, etc. These recently developed processes for preparing leather replacement compositions do not, however, provide products which are satisfactorily resistant to fuzzing upon being subjected to scuffing or abrasion.

An object of the present invention, therefore, is to provide a leather replacement composition having outstanding resistance to surface fuzzing upon being abraded. A still further object is to provide a process of preparing such leather replacement compositions. The foregoing and other objects will more clearly appear hereinafter.

These objects are accomplished by the present invention which, briefly stated, comprises forming a fibrous, substantially water vapor-impermeable sheet comprising a base stratum of uniformly dispersed structural fibers, a surface stratum of uniformly dispersed soluble pore-forming fibers free of structural fibers, said pore-forming fibers being soluble in a solvent which is a non-solvent for the structural fibers, said strata being impregnated with thermoplastic, soft, elastomeric polymeric binder material to form a composite sheet, treating said sheet to cause said structural fibers to break away from said binder, and dissolving out the soluble pore-forming fibers, whereby to form a water vapor-permeable sheet of polymeric binder material having a porous surface stratum free of structural fibers and a base stratum having structural fibers and contiguous channels distributed therethrough.

The term "contiguous channels," as applied to the interconnecting pores formed in the fiber-reinforced strata of the leather replacement sheets of this invention, means that the channels or pores are immediately adjacent the structural fibers. It should be emphasized that the pores or channels are not necessarily wholly annular; that is, the structural fiber is not necessarily entirely broken away from the surrounding binder polymer. In some cases, for example, a continuous pore or capillary may spiral around a continuous length of fiber; whereas, on the other hand, the capillary, formed by the fiber's breaking away from the surrounding binder polymer, may take the form of a "hairline crack" running substantially parallel and immediately adjacent a structural fiber.

Any convenient known expedient for treating the initial sheet to cause the structural fibers to break away from the polymeric binder material to form contiguous channels in the base stratum may be employed. Thus, by selecting relatively non-extensible structural fibers and a binder polymer which is extensible relative to the structural fibers, stretching the resulting sheet in one or both directions will serve to break the embedded fibers away from the binder polymer and form contiguous channels in the sheet upon removal of the stretching forces, i. e., relaxation. Such a process is disclosed and claimed in the copending application of V. L. Simril, U. S. Serial No. 318,732, filed November 4, 1952. The process comprises forming a substantially water vapor-impermeable composite sheet by impregnating a non-

woven sheet of fibers of substantially water vapor-impermeable, substantially non-extensible material with substantially water vapor-impermeable, relatively extensible binder polymer, said binder polymer constituting from about 30% to about 70% by weight of the total weight of fibers and binder polymer, and stretching said composite sheet whereby to form a water vapor-permeable sheet. In general, the extent of stretch in one or two directions, and the degree of adhesion between fiber and binder affects the size of the channels or pores formed adjacent the fibers, i. e., the degree to which the channels approach a wholly annular form.

The expression "relatively extensible material," as used herein, means that the material must be stretchable under the stretching forces to be employed and must elongate during the stretching and substantially recover upon releasing the stretching forces. The expression "relatively non-extensible material" means that the material stretches to a substantially lesser extent, if at all, than the "relatively extensible material" under the stretching forces imposed.

The steps of swelling and deswelling (shrinking) structural fibers in a fiber-reinforced polymeric sheet or film also result in breaking the embedded fibers away from the binder polymer, i. e., breaking the adhesive bonds between fibers and binder; and this also forms interconnecting contiguous channels or pores in the sheet. The swelling-deswelling treatment is disclosed and claimed in copending application Serial No. 325,689, J. C. Richards, filed December 12, 1952, now abandoned. This process comprises associating liquid-swellable structural fibers and soft, initially thermoplastic polymeric binder material having a softening temperature below the softening temperature of said fibers to form an initial sheet, hot-pressing the initial sheet at a temperature above the softening temperature of said binder and below the softening temperature of said fibers, whereby to form an essentially impermeable composite sheet, soaking said composite sheet at a temperature between the softening temperature of said binder and of said fibers in a liquid which swells said fibers, and thereafter drying the sheet at a temperature which is no greater than the softening temperature of the binder polymer and is usually below the softening temperature of the binder polymer. The degree to which the contiguous channels or pores therein approach a wholly annular form depends mainly upon the degree to which the fibers are swollen and the strength of the adhesive bonds between fibers and binder.

The term "liquid swellable fiber" as employed herein denotes fibers which swell in contact with a liquid by absorption of the liquid into the fibers and which, upon removal of the liquid by drying, shrink back to substantially their original dimensions. The liquid used should not dissolve the binder material although it may be absorbed to a limited extent by the binder. On the other hand, the liquid employed may or may not act as a solvent upon the pore-forming fibers. When the liquid is a solvent for the pore-forming fibers, the step of swelling the structural fibers and extracting the pore-forming fibers may be carried out in a single step.

The "softening temperature" of the thermoplastic binder polymer is the "second order transition temperature" ( $T_m$ ) in the case of a normally amorphous polymer; or, in the case of a crystalline polymer, the softening temperature is the beginning of the melting point range or the temperature at which the crystalline phase begins to disappear at an appreciable rate, as determined by X-ray examination or other suitable technique. The "second order transition temperature" of an amorphous polymer is defined as the temperature at which a discontinuity occurs in the curve of a first derivative thermodynamic quantity of the polymer with temperature. It can be observed from a plot of density, linear expansion, specific volume, specific heat, sonic modulus or index of refraction against temperature. United States

Patent No. 2,556,295 to Pace discloses specific steps involved in measuring the second order transition temperature of an amorphous polymer. Copending application U. S. Serial No. 325,689, filed December 12, 1952 in the name of J. C. Richards, also discloses a procedure of measuring the second order transition temperature of an amorphous polymer. In the case of a crystalline polymer, the softening point thereof, as related to the temperature at which the swelling step of the present process is carried out, is the temperature at the lower end of the melting point range. This temperature is further defined as the lowest temperature at which the crystalline structure begins to disappear at an appreciable rate, as measured by any of the known techniques such as X-ray examination, infra-red studies, or by the measure of heat content as carried out by Raine, Richards, and Ryder and reported in Transactions of the Faraday Society, 41, 61 (1945). In this study, for example, a sample of polyethylene was found to have a melting point range from 90° C. to 104° C.; i. e., at 90° C., half of the crystalline structure remained.

Subjecting a fiber-reinforced sheet to a combination of swelling-deswelling and stretching, such as is disclosed and claimed in the copending application of Harold L. Mighton, Serial No. 430,550, filed May 18, 1954, is more effective than either stretching alone, or swelling and deswelling alone, for breaking the bond between fibers and binder polymer, since such a combination process serves to create a greater volume of void space in the treated sheet; i. e., the contiguous channels or pores formed are more advanced toward a wholly annular form than contiguous channels or pores formed by either stretching alone or swelling-deswelling alone.

In general, the leather replacement sheets of the present invention are prepared by forming a substantially water vapor-impermeable, compacted sheet of a polymer reinforced with structural fibers and having integral surface strata containing uniformly dispersed pore-forming fibers, but no structural fibers, and thereafter treating the said water vapor-impermeable sheet by stretching the sheet and/or soaking the sheet in liquid which swells the fibers, and finally extracting the soluble pore-forming fibers from the surface strata.

The expression "substantially water vapor-impermeable" as applied to the initial composite sheet (i. e., before treating) means that the sheet has a leather permeability value (LPV) of less than 1,000 grams/100 sq. meters/hour, measured at 23° C. and 90% relative humidity. In general terms which may be applied to any combination of relatively extensible and relatively non-extensible materials useful in the present process, the water vapor permeability of the initial composite base sheet is substantially no greater than that of a homogeneous sheet of the relatively extensible material or the relatively non-extensible material, whichever has the higher water vapor permeability. Usually, providing the initial composite base sheet is prepared in such a manner that there are substantially no voids present in the sheet, the water vapor permeability of such a base sheet is intermediate between the permeabilities of homogeneous sheets of the two major components of the base sheet. Actually, the leather permeability values (LPV) of the initial compacted, substantially water vapor-impermeable sheets which are transformed into permeable sheets by following the present process are low not only because the sheet is compacted by hot-pressing, but also because of the thickness of the sheets which are useful for converting to leather replacement sheets. That is, the initial sheets are usually between 0.015"-0.05" in thickness, and homogeneous sheets of either the binder polymer or the structural fiber having thicknesses within this range also have low LPV's. Normally, the LPV is appreciably less than 1,000, and in no case greater.

A clearer understanding of processes of forming the leather replacement compositions of the present invention

and the structure of the compositions themselves may be had by referring to the accompanying drawings wherein:

Figure 1 is a flow diagram of a process of making the present leather replacement sheets by stretching a hot-pressed sheet comprising structural fibers, a binder polymer and strategically positioned, that is, positioned in a surface stratum, soluble pore-forming fibers, and thereafter extracting the pore-forming fibers;

Figure 2 is a flow diagram of the necessary steps of another embodiment of the process of this invention, namely, one involving simultaneously or separately swelling structural fibers and extracting strategically positioned, that is, positioned in a surface stratum, pore-forming fibers by immersing the initial sheet in a liquid, and thereafter deswelling the structural fibers by drying the resulting sheet to remove liquid from the structural fibers; and

Figure 3 represents a flow diagram of a series of steps leading to the preparation of the present leather replacement composition wherein alternative steps for preparing the substantially impermeable, initial compacted sheet are presented, and the initial sheet is made porous by a combination of stretching and extraction or by a combination of swelling-deswelling and extraction.

In referring to the accompanying flow diagrams, it should be understood that the cross-sections of typical "lay-ups" and sheets (in various stages) represent a minimum structure. In other words, stage A of Figure 1 illustrates compositing three essential types of strata, namely, a layer of pore-forming fibers (layer 6), a layer of binder polymer (layer 4), and a layer of structural fibers (layer 2). These layers may vary considerably in thickness, this depending on the thickness of the ultimate desired leather replacement sheet. On the other hand, as many additional alternate layers of binder polymer and structural fibers as practicable may be included in the initial lay-up, as will be illustrated in the examples to be presented hereinafter.

The nature of the initial fibrous polymer sheet, that is, the relative positions and distribution of structural and pore-forming fibers, determines the properties of the final leather replacement compositions. A "lay-up" or composite of essential components is shown in stage A of Figure 1. That is, a web of structural fibers 1, for example, nylon fibers, forms the lower layer, layer 2. On top of this mat or sheet of non-woven fibers is placed a homogeneous sheet of a binder polymer 3, layer 4, for example, a blend of polyethylene and polyisobutylene (50/50). Finally, layer 6 is placed upon the composite, layer 6 being a web of pore-forming fibers only. The "lay-up" may, of course, be comprised of a plurality of layers of each type so long as the stated relative disposition of structural and pore-forming fibers is maintained. Step 1 consists of placing the composite between two layers of non-heat-sealing cellophane (not shown) and hot-pressing the composite at a temperature sufficient to cause the binder polymer to flow and thoroughly impregnate the fibrous components, the temperature not being sufficiently great to fuse or transpose the fibers to any appreciable degree. At stage B, the resulting compacted structure is a film or sheet of the binder polymer reinforced with structural fibers and having integral surface strata containing pore-forming fibers, but no structural fibers. Step 2 involves stretching the sheet of stage B in one or two directions, the film being elongated anywhere from 10 to 50% in one or both directions, that is, in directions perpendicular to each other. This stretching step is embodied in the process of Simril, described and claimed in copending application U. S. Serial No. 318,732. In stage C, the fiber-reinforced film is porous as a result of the stretching step. That is, the stretching has served to stretch the binder polymer to a greater extent than the embedded fibers so that the binder polymer has been broken away from around the fibers; and interconnecting channels or pores 7 contiguous with the

fibers have been formed in the film or sheet. However, in stage C, the upper surface still contains the pore-forming or extractable fibers. Hence, upon abrasion, the surface of this composition would fuzz because the abrading action would raise the fibers to the surface in the form of fuzz. Therefore, step 3 involves extraction of the pore-forming fibers from the surface of the porous sheet of stage C, whereby to form pores 8 in the surface stratum of the sheet. It is important to emphasize that this extraction process may be carried out relatively rapidly compared with the extraction of soluble fibers from within a fiber-reinforced sheet containing soluble fibers throughout the entire cross-section. This is because the solvent penetrates rapidly into the shallow surface strata containing the soluble fibers. Furthermore, stretching the sheet prior to extraction facilitates rapid penetration of solvent into the sheet. Stage D, therefore represents a porous fiber-reinforced polymer film having integral porous surface strata having no fibers.

Referring to Figure 2, another process of preparing compositions of the present invention is illustrated. Stage A represents a composite or aggregation of essential components, as in Figure 1, wherein layer 2 is a non-woven fibrous mat of a structural fiber 1, for example, nylon fibers. Layer 4 is a homogeneous film of a binder polymer 3, for example, polyethylene or a melt blend of polyethylene and polyisobutylene. Layer 6 is a non-woven fibrous mat of extractable or pore-forming fibers 5, for example, in this illustration, polyvinyl alcohol. The composite of stage A is then hot-pressed in accordance with step 1 to cause the binder polymer to flow around the lattice of structural and pore-forming fibers to impregnate the fibers. The compacted sheet of stage B is an impermeable, that is, substantially impermeable to water vapor and air, polymeric film or sheet reinforced with structural fibers and having the upper surface stratum containing extractable pore-forming fibers. Step 2 involves immersing a compacted sheet of stage B into a hot liquid medium at a temperature above the softening temperature of the binder polymer, for example, hot water when polyvinyl alcohol is the composition of the pore-forming fibers, which medium serves to swell the structural fibers and extract the pore-forming fibers from the upper surface stratum of the sheet. Stage C illustrates the condition of the soaked sheet immediately after removing the sheet from a hot liquid medium. In stage C, the upper surface stratum is porous (pores 8), i. e., is devoid of pore-forming fibers; and the structural fibers in the lower portion of the sheet are swollen by the absorbed water. Furthermore, the polymer binder is considerably softened as a result of being soaked in a liquid medium at a temperature above the softening temperature of the binder. Step 3 involves drying or removing the liquid medium from the structural fiber at a temperature below the softening temperature of the binder polymer. The resulting product of stage D is porous throughout as a result of a deswelling of the swollen structural fibers; that is, the structural fibers shrink to their normal dimensions when the sheet is cooled and dried at a temperature below the softening temperature of the binder polymer. Shrinkage (deswelling) of the structural fibers away from the adjacent hardened polymeric binder polymer (the softened, i. e., softened during soaking in a hot liquid, binder polymer is deformed when the structural fibers are swollen) results in forming channels or pores 7 contiguous with the structural fibers, thereby forming a porous structure. Hence, stage D illustrates a porous fiber-reinforced polymer film or sheet having an integral porous surface stratum containing no fibers.

It should be emphasized that other procedures may be employed for fabricating an initial composite sheet having soluble fibers strategically positioned in the surface stratum, such sheet being readily convertible into a porous fiber-reinforced sheet having integral a porous sur-

face stratum substantially free of fibers. Figure 3 illustrates the series of steps required to form, by a somewhat different procedure than that illustrated in Figures 1 and 2, a leather replacement composition of the present invention by a combination of extraction and stretching or extraction of pore-forming fibers and swelling-deswelling of the structural fibers, for example, structural fibers of nylon. The superimposed mats 9 and 10 of structural fibers 11, shown in stage A, are impregnated (step 1) by conducting the mats through a solution containing a suitable polymer 12; the polymer may be dissolved in a solvent; or the polymer may be dispersed in a non-solvent medium. Stage B illustrates the superimposed webs after having been impregnated with a polymer. Step 2 involves hot-pressing the impregnated mats to compact the sheet. Since pore-forming fibers are to be pressed into the upper surface stratum of the sheet, this initial compacting step should not be carried out at a temperature high enough to cure the binder, that is, when a curable binder is used. Stage C represents the compacted fiber-reinforced impermeable sheet. Step 3 involves coating the compacted sheet with, for example, a dispersion of pore-forming fibers 13 in a non-solvent medium, which may or may not contain a dissolved polymer. This leads to stage D, which shows the compacted fiber-reinforced polymeric sheet having pore-forming fibers deposited as a surface stratum 14. This composition is then subjected to step 4 which involves hot-pressing the pore-forming fibers into the surface stratum of the sheet, and completing the compacting of the sheet. The resulting product is illustrated as stage E. In accordance with the procedures described in Figures 1 and 2, the product in stage E may be subjected to a stretching step, that is, stretching in one or both directions to form a product in stage F. The product of stage F is permeable to water vapor and air, but still contains pore-forming fibers in the surface stratum. Consequently, the product of stage F is subjected to an extraction step which removes the soluble fibers from the surface stratum. Hence, stage G represents a fiber-reinforced porous sheet or film having a porous surface stratum free of fibers. On the other hand, the sheet of stage E may be subjected to a simultaneous extraction and swelling step by immersing (step 5A) the sheet in a liquid (at a temperature above the softening temperature of the binder polymer) which dissolves the pore-forming fibers and swells the structural fibers. As the net result of such a step, stage F represents a sheet having the pore-forming or soluble fibers removed from the surface stratum and having the structural fibers in swollen form. This product is then cooled and subjected to a drying step at a temperature below the softening temperature of the polymeric binder to remove the swelling liquid from the structural fibers to permit them to return to their original dimensions. Hence, stage G represents a porous fiber-reinforced film or sheet having a porous surface stratum containing no fibers.

As an alternative procedure of depositing pore-forming fibers upon the surface of compacted fiber/binder sheet, i. e., step 3 of Figure 3, the fibers may be deposited from a solution containing a dissolved polymer wherein the pore-forming fibers are present as a dispersed phase. For example, polyethylene may be dissolved in hot toluene, and polyvinyl alcohol pore-forming fibers may be present as a dispersed phase. Upon coating the surface of a compacted fiber/binder sheet with this composition and evaporating the solvent, the coating takes the form of a film of polyethylene having fibers of polyvinyl alcohol dispersed therein. The coated fiber/binder sheet is then consolidated by hot-pressing the sheet, and the coating becomes integral with the sheet providing there is sufficient adhesion between the polymer of the coating and the binder polymer of the initial fiber/binder base sheet. This procedure serves a dual purpose in that it provides a method of strategically distributing pore-forming fibers in the surface stratum of a sheet, and it

provides a method of preparing a porous fiber/binder composition having a surface which is harder, tougher and more resistant to destruction by scuffing or abrasion than the binder polymer in the internal structure of the sheet. On the other hand, the binder in the internal structure is much more pliable and flexible than the binder in the surface stratum, the overall structure being highly flexible but having desirable surface properties. It should be emphasized that the binder employed in the surface stratum must adhere strongly to the internal binder. For example, polyisobutylene may be employed as the internal binder, and polyethylene may be employed in the surface stratum; and since polyisobutylene and polyethylene adhere strongly under heat and pressure, an integral structure is formed after the coated sheet is consolidated.

Although it is most expedient in treating the initial compacted (substantially impermeable) sheet to extract soluble pore-forming fibers and swell the structural fibers simultaneously, i. e., the sheet is immersed in a liquid which simultaneously extracts pore-forming fibers and swells structural fibers, the sheet may be immersed first in a non-solvent medium to swell structural fibers, dried to deswell (shrink) the fibers, and finally immersed in a solvent to extract pore-forming fibers. On the other hand, the pore-forming fibers may be extracted prior to stretching the sheet, but preferably the stretching step is carried out first because it opens pores in the sheet, and this obviously facilitates penetration of solvent for extracting pore-forming fibers from the surface stratum.

Furthermore, it should be pointed out that it may be advantageous under certain circumstances to stretch the compacted sheet first to only a slight degree, i. e., 10-20% in one or two directions, in order to open the structure of the sheet and facilitate penetration of the solvent into the surface stratum. This step may then be followed by extraction of pore-forming fibers from the surface stratum, and thereafter completion of the stretching step by stretching the extracted sheet an additional 30-40% in one or two directions.

As described hereinbefore with reference to the accompanying diagrams in the form of flow charts, the particular process steps which may be employed to produce a particular substantially non-fuzzing leather replacement composition of the present invention may be varied. In all cases, however, it is essential that a pore-forming fiber be incorporated into the surface stratum of the initial composite sheet before the sheet is subjected to any of the basic processes or combinations thereof described hereinbefore. In all cases, prior to subjecting the initial impermeable composite sheet to the process steps which impart permeability thereto, the initial composite sheet must be compacted to form a fiber-reinforced polymer sheet or film wherein the binder polymer completely surrounds or impregnates each individual fiber of the fibrous components. This is accomplished by forming a lay-up or composite of the essential components of the fiber-reinforced sheet, it being essential that these components be composited in a strategic order for the purpose of placing the particular type of fibers, that is, the structural and pore-forming fibers, in particular positions throughout the cross-section of the sheet for the purpose of producing a porous fiber-reinforced composition having interconnecting pores contiguous with the fibers which are distributed substantially uniformly throughout the sheet below the fiber-free surface stratum. It is obvious that in every case a layer of pore-forming fibers must be strategically positioned in the initial composite, that is, before final compacting, so that the compacted sheet contains pore-forming fibers distributed uniformly in the surface stratum thereof. Obviously, it is entirely within the scope of the present invention to incorporate pore-forming fibers in both the upper and lower surface strata of a compacted sheet so that the ultimate water vapor-permeable composition

has both surfaces which are porous but free of structural fibers. It is also essential in preparing the leather replacement compositions of the present invention to position the structural fibers in the initial composite sheet so that, after compacting, the structural fibers are uniformly distributed throughout the cross-section of the compacted sheet, but are absent from the surface strata which contain solely the pore-forming fibers. Techniques of accomplishing the strategic positioning of various types of fibers along with suggested processes of impregnating these fibers with a polymeric binder have been illustrated hereinbefore with reference to the accompanying diagrams.

As mentioned above, the initial composite (uncompacted) sheet is subjected to a hot-pressing or consolidating operation which causes the binder polymer to melt and flow, this resulting in thoroughly impregnating the fibrous components therein and redistributing the polymeric binder to form a continuous solid polymeric film or sheet. The hot-pressing step must be carried out at a temperature above the flow temperature of the polymeric binder (flow temperature, for example, may be determined by ASTM test D-569-48) and below the deformation or softening temperature of the fibrous components. Generally, the compositions are hot-pressed at a temperature within the range from 120°-200° C. under pressures varying from 50 pounds per square inch to 2,000 pounds per square inch. In all cases, the temperature at which the fiber/binder sheet is consolidated must be below the degradation temperatures of the fibrous components and the binder polymer. During the hot-pressing step, the fibrous components, which must not be deformed to such an extent as to lose their identity as fibers, or be transposed to the extent that a considerable portion of fibers are more concentrated in one portion of the sheet than in others, serve as a lattice around which the polymeric binder flows to impregnate each and every fiber. Hence, after consolidation, the sheet takes the form of a fibrous lattice which is completely embedded or surrounded by the binder polymer. In this form, the compacted fiber-reinforced polymeric film or sheet is ready to be treated by one or combinations of the basic processes, e. g., extracting stretching, and swelling-deswelling, to impart permeability thereto.

It is in the binder material that the interconnecting capillaries or pores are formed by treatment by one or more of the above processes. By extracting the soluble or pore-forming fibers from the surface stratum, interconnecting pores or capillaries having substantially the same shape as the soluble fibers are formed. On the other hand, the process of stretching a fiber-reinforced sheet, which is more fully described in the above mentioned copending application U. S. Serial No. 318,732, produces a fiber-reinforced sheet having channels or capillaries contiguous with each structural fiber which has been broken away (the adhesive bond between the structural fiber and the binder polymer has been broken) from the binder polymer. The technique of swelling-deswelling of the structural fibers also serves to break the adhesive bond between the structural fibers and binder polymer; and, consequently, the channels or capillaries formed are also contiguous with the structural fibers. It is also the binder polymer which holds together and is reinforced by the structural fibers. Generally, the binder polymer may be selected from a great variety of soft, elastic, initially thermoplastic, synthetic polymers which include polymers generally classified as elastomers. The polymeric binder, in general, should be tough, pliable, and elastic; and it should be at least initially thermoplastic and should melt and flow at a temperature below the deformation (softening) temperatures of the structural fiber and pore-forming fiber. By the term "initially thermoplastic" is meant that the binder material must melt and flow under the conditions of the hot-

pressing step. When the binder material is in the form of individual fibers, the length of the fibers has no effect upon the properties of the extracted sheet, provided that the binder fibers have been strategically uniformly dispersed through the composition before heat and pressure are applied.

In describing the binder material as a tough, pliable, at least initially thermoplastic polymer, the following more specific requirements apply to those binder materials that are preferred.

1. Tensile strength should be at least 500 p. s. i.
2. The elongation must be at least 100%.
3. Materials not having a tensile strength and elongation greater than the above minimum specifications may be satisfactory if the product of their tensile strength and elongation (where 100% equals 1) is at least 1,000.
4. The tensile modulus must not be more than 25,000 p. s. i. and, preferably, not more than 5,000 p. s. i.

A number of specific thermoplastic binder polymers useful for purposes of this invention and classified as elastomers are disclosed by H. L. Fisher (Industrial and Engineering Chemistry, August 1939, page 942). The binder polymer employed should be chemically dis-

similar to the structural and pore-forming fibers. Because of their readier availability, better properties, and appreciably better ease of handling, the addition polymers are preferred. A particularly outstanding group are the addition polymers containing in combined form

the ethylenically unsaturated monomers including both the mono- and diene-type monomers. The most outstanding group of these addition polymeric binders are the vinylidene polymers and copolymers including both the monoene and diene types. This class of polymers

is characterized by having in each polymerizable monomer therein involved as the only polymerizable ethylenic unsaturation, terminal ethylenic groups wherein the terminal carbon is a methylene carbon, i. e., those containing one or more vinylidene ( $\text{CH}_2=\text{C}-$ ) groups. Included in this most preferred class are the great majority

of commercially available addition polymers. Specific examples of such polymers include the various vinylidene hydrocarbon polymers such as butadiene/styrene, polyethylene, polyisobutylene, polyisoprene, both synthetic

and natural; the various negatively substituted polymers such as the vinylidene halide including vinyl halide polymers, e. g., polyvinylidene chloride, polyvinyl chloride and polyvinyl fluoride; derivatives of such polymers as halogenated vinyl and vinylidene polymers, e. g., chlorinated polyethylene, and chlorinated polyvinyl chloride;

the various vinylidene polymers wherein one or both of the indicated free valences of the 2-carbon of the vinylidene group are bonded directly to carboxyl groups or groups hydrolyzable to carboxyl groups either directly to the acyl carbon or the oxy oxygen thereof, such as polymers of various vinylidene esters, including vinyl acetate and ethylidene diacetate; vinylidene carboxylic acids and their derivatives such as acrylic acid, acrylonitrile, and methacrylamide. Also included in this most preferred

group are the various copolymers of such vinylidene monomers, including specifically the various monoene and diene copolymers of this class such as 2,3-dichlorobutadiene-1,3/2-chlorobutadiene-1,3 copolymers; the various monoene/vinylidene copolymers such as the commercially important vinyl and vinylidene chloride copolymers, e. g., vinyl chloride/vinyl acetate, vinyl chloride/vinylidene chloride, and vinyl chloride/vinyl acetate/acrylonitrile copolymers; the various vinylidene hydrocarbon negatively substituted vinylidene copolymers,

e. g., ethylene/vinyl acetate and the hydrolyzed products therefrom; ethylene/vinyl chloride, and butadiene/acrylonitrile copolymers.

In the case of those binder components containing in combined form appreciable proportions of diene monomers, particularly the vinylidene diene monomers, it is

frequently desirable to have present in the solution, dispersion, or bulk treating material, whichever is used, suitable amounts of chemical agents for effecting under controlled conditions, after the fiber has been impregnated with the binder and the whole mat suitably compacted, the cross-linking of the diene copolymer component. These chemical systems for effecting such controllable cross-linking are well known in the rubber art and, in the case of the diene hydrocarbon polymers and copolymers, such as 2-chlorobutadiene-1,3(chloroprene), normally function through a disulfide formed cross-link arising from the presence of mercaptans and/or sulfur in the diene polymer composition; and in the case of such polymers as chlorosulfonated polyethylene, curing may be carried out in the presence of metallic oxides such as zinc or magnesium oxides.

Various polyesters containing terephthalic acid or derivatives thereof as essential components are also useful as binder polymers, these including polyethylene terephthalate and copolymers made from ethylene glycol, terephthalic acid and sebacic acid of the general type described and claimed in United States Patents Nos. 2,623,031 and 2,623,033 in the name of M. D. Snyder. Polyamides useful as a binder polymer include N-methoxymethyl polyhexamethylene adipamide and other similar polymers disclosed and claimed in United States Patent No. 2,430,860. Also included among useful binder polymers are the polyvinyl acetals, such as polyvinyl butyral, polyvinyl laural, etc. Included among various elastomeric polymers which may be employed as binders in the present invention are the polyurethanes which are essentially reaction products of (1) an organic polyisocyanate or polyisothiocyanate with (2) a compound obtainable by reacting (a) one or more polyhydric alcohols with (b) one or more polycarboxylic acids (either in the presence or absence of one or more monocarboxylic acids). Specific products of this type are described and claimed in United States Patent No. 2,333,639 to R. E. Christ and W. E. Hanford.

Other types of elastomeric polymers which may be used as binders include reaction products of polyalkylene ether glycols and organic diisocyanates.

As pointed out previously, a critical factor in the choice of a preferred polymeric binder is the fact that it should not be chemically similar to the structural fiber. This is quite important since it has been found that where the polymeric binder is chemically similar to the structural fibers, the resulting sheet material, while occasionally adequate in tensile strength, is generally deficient in drape, hand, and flex life, and, more importantly, is usually particularly deficient in tear strength. A convenient rule for characterizing the chemically dissimilar polymeric binders is that they be incompatible in the melt with the polymer from which the structural fibers are formed.

In many instances, it is desirable to have present in the binder composition appreciable proportions of plasticizers, now well known in the art, for the binder polymers. This is particularly important in the case of the vinylidene resins, to prevent formation of products of too great stiffness, especially with the higher molecular weight, negatively substituted vinylidene polymers and copolymers, such as the vinyl chloride/vinylidene chloride and vinyl chloride/vinyl acetate copolymers, so as to produce leather-like products of good drape and high pliability. Suitable examples of these include the higher molecular weight mono- or dicarboxylic acid/alcohol or polyolesters such as glycerol mono-oleate, glycerol sebacate, dioctyl phthalate, and ethylene octanoate; or the lower molecular weight polyesters and polyethers such as the polyalkylene oxides and their esters, e. g., polyethylene oxide, methoxy-polyethylene glycol; and the lower molecular weight condensation polyesters such as polyethylene glycol adipate.

The binder material may be incorporated into the ini-

tial impermeable composite sheet in a variety of ways, several of which have been illustrated hereinbefore. The binder material may be in the form of fibers which may be carded along with the structural fibers and the pore-forming fibers to form a composite sheet by pressing the carded mixed fibers at elevated temperatures. Webs or mats of mixtures of structural fibers, pore-forming fibers and binder polymers may be formed by mutual coagulation of a mixed dispersion of the three components. A fibrous mat of a mixture of structural and pore-forming fibers may be impregnated by dipping or spraying with a binder polymer which may be dispersed in a nonsolvent, e. g., aqueous medium, or may be in a solvent solution. On the other hand, a fibrous mat containing both structural and pore-forming fibers or just structural fibers may be impregnated with a binder polymer in the form of a hot melt. A fibrous mat of structural and pore-forming fibers or structural fibers alone may be impregnated with a binder polymer by calendering techniques or by spraying the binder material from an aqueous dispersion or solvent solution onto one or both sides of the fibrous mat, followed by the application of heat and pressure to impregnate the fibrous portion of the mat with the binder material. Regardless of the technique employed to form a composite sheet, the sheet is compacted prior to extraction of the soluble or pore-forming fibers by pressing at a temperature above the flow temperature of the binder and below the softening or deformation temperature of the structural fiber and pore-forming fiber.

30. The binder polymer in the surface stratum of the leather replacement compositions of this invention may be different from the binder polymer of the internal or base strata. The purpose of this is to obtain a sheet having maximum flexibility and maximum surface hardness and resistance to destruction upon scuffing or abrasion. The binder polymers must adhere strongly to each other in order to form an integral sheet upon consolidation of the sheet under heat and pressure. Still another means of obtaining a highly flexible leather replacement having a surface which is hard, tough and resistant to destruction on abrasion is to employ the same binder polymer throughout the composition, but employ homogeneous sheets or films of the binder polymer (in the initial lay-up) containing varying amounts of a plasticizer. For example, the 35. sheets or films of binder polymer in the internal structure may contain as much as 50% plasticizer while the uppermost sheet of binder may be unplasticized.

Any fiber having substantial strength and which is substantially insoluble in the solvent employed to extract 40. the pore-forming fibers of the surface stratum of the sheet may be employed as the structural fiber. Fibers of nylon, i. e., synthetic linear polyamides such as polyhexamethylene adipamide, polyhexamethylene sebacamide, polycaproamide and interpolyamides, etc., are out-

45. standing for use as the structural fibers in the leather replacement compositions of the present invention. The use of nylon structural fibers produces a porous composition having high tear strength, tensile strength, softness and flex life. In general, however, resultant superior physical 50. properties are obtained when the structural fibers are oriented synthetic linear condensation polymers, e. g., the polyamides, the polyesters, polyesteramides, mixtures or blends thereof, such as the dibasic acid/diamine or amino acid polyamides, the dibasic acid/diol or hydroxy acid/polyesters, or the intermixed polyester/polyamide products by now well known in the art and described in greater detail in United States Patents Nos. 2,071,250, -251, -253, 2,130,948, 2,224,037, 2,572,844, and the like. The length of the structural fibers may be varied according to the 55. general strength of properties required. Structural fibers as short as 0.01" may be employed, but structural fibers having a length of about 1.5" give a product of substantially optimum strength properties. Using structural fibers longer than 1.5" imparts little additional strength 60. to the present leather replacement compositions; but, as 65. 70. 75.

mentioned hereinbefore, it may be convenient to use longer fibers; and the use of longer structural fibers, e. g., up to 8", is within the intended scope of the present invention. On the other hand, structural fibers less than 0.01" in length add little to the strength of the sheet over that of a sheet composed wholly of the binder polymer.

Other types of structural fibers which may be used, particularly in the form of mixtures with polyamide, polyester, or polyesteramide type fibers, include fibers of cotton viscose and acetate rayon, wool, polyacrylonitrile, acrylonitrile copolymers, polyvinyl acetals, and glass. It should be emphasized that a considerable advantage may be gained by employing mixtures of different types of structural fibers, the particular mixture depending upon the particular combination of process steps to be used in making the initial compacted sheet porous. For example, if a combination of swelling-deswelling and extraction is to be carried out, there is an advantage in employing a quantity of structural fibers which are more readily swollen by water than nylon fibers, for example, viscose fibers. Hence, a mixture of viscose rayon and nylon fibers may be advantageous, or, mixtures of viscose rayon and polyethylene terephthalate fibers, or mixtures of all three.

The pore-forming fiber is usually a staple fiber; that is, it should be adaptable to making mats. In this form, the pore-forming fiber is randomly disposed in the surface strata, and extraction thereof results in the formation of a network of interconnecting capillaries or pores. Furthermore, the pore-forming fiber must not be excessively softened at the flow temperature of the binder and must be readily extractable from the composite sheet with a solvent which is substantially inert, i. e., has no solvent action, toward the structural fiber and the binder material. Cellulose acetate fibers are readily extractable using acetone, and some grades of polyvinyl alcohol are readily extractable with water. Other suitable pore-forming fibers are those of sodium alginate, potassium metaphosphate polymer, glass, and carboxymethyl cellulose.

Products of satisfactory leather permeability may be formed using pore-forming fibers as short as 0.01", e. g., 0.01" cellulose acetate flock. However, a considerable increase in leather permeability is realized when longer pore-forming fibers are employed. For example, increasing the length of the pore-forming fiber from 0.01" up to a length of 0.25" produces a substantial increase in the leather permeability of the resulting product. However, an increase in pore-forming fiber length from 0.25" to 0.5" generally results in substantially no increase in the leather permeability of the resulting sheet.

Variations in the denier of the structural fibers and pore-forming fibers appear to have little effect upon leather permeability. On the other hand, it has been found that decreasing the thickness of the pore-forming fiber results in forming a leather replacement sheet having improved resistance to penetration by liquid water. In general, it may be said that fibers which are finer than one denier are difficult to process on standard textile machinery. Furthermore, the greater the fiber denier, the greater is the tendency of the fibers to shift within the binder under tearing and flexing, this action in general making the product more durable. At the other extreme, fibers coarser than 16 denier are extremely harsh and more closely resemble bristles.

The choice of a solvent for extracting the pore-forming fiber from the surface stratum of initial impermeable sheet depends upon the particular pore-forming fiber and the nature of the structural fiber and the binder material. The solvent should be one in which the pore-forming fiber is readily soluble; and it should be substantially inert, i. e., have no solvent action, toward the structural fiber and the binder material. The duration of the extraction step depends upon the weight of the pore-forming fiber in the initial sheet, the thickness of the surface stratum containing the pore-forming fibers, the solubility

of the pore-forming fiber in the solvent, the temperature of the extracting liquid, and the degree of agitation, and the ease with which the solvent can penetrate the sheet. It is within the scope of the present invention to employ a liquid (as a solvent) which degrades the pore-forming fibers, while not affecting the structural fibers or binder polymer, but which liquid dissolves the degradation product, that is, dissolves the degraded pore-forming fibers and thereby extracts them from the fiber/binder sheet. On the other hand, the fibers may be degraded with an acidic or basic liquid followed by the step of dissolving out the degraded fibers with another liquid such as water.

On the basis of numerous types of wearing comfort tests, it has been ascertained that membranes, e. g., leather and leather replacements, exhibiting a leather permeability of 2,000 to 10,000 grams/100 sq. meters/hour would provide wearing comfort equivalent to that obtained with glazed leathers and heavy shoe upper leathers. Furthermore, permeabilities of 10,000 to 22,000 were found to provide adequate wearing comfort equivalent to that obtained with the lightest shoe leathers.

In preparing the leather replacement compositions of this invention in accordance with a stretching-extraction technique or by the process of swelling-deswelling and extraction, the weight ratio of binder polymer to structural fiber in the initial substantially impermeable compacted sheet may vary from 30:70 to 70:30. However, the optimum quantity of binder material in the initial composite sheet ranges from 40 to 60% based upon the total weight of the two major components, that is, the binder and the structural fibers. In each case, the pore-forming fibers are uniformly distributed only within the surface stratum; and the weight of these soluble pore-forming fibers normally ranges between 5% and 25%, based upon the total weight of the fibrous components in the sheet. Normally, the densities of the binder polymer and the structural and pore-forming fibers are relatively close; and in such cases, the ratio of the components may be expressed on either a volume or weight basis. Generally, as the quantity of binder polymer in the composition is reduced, the initial composite compacted sheet becomes more and more permeable to water vapor (the stretched sheet or a sheet subjected to swelling-deswelling is highly permeable by comparison); but other properties (particularly strength) and characteristics of the final sheet, i. e., the stretched sheet or one subjected to swelling-deswelling, are not satisfactory for use as a leather replacement, for example, in boots, shoes, gloves, chair coverings, etc. Compositions containing too low a quantity of binder material feel more like felt instead of leather, and the tensile strength and tear strength are appreciably below the tensile and tear strength of similar compositions having from 40-60% of the binder polymer present. This is because in most cases the amount of binder polymer is insufficient to hold the structural fibers together. On the other hand, as the amount of binder polymer is increased, the initial composite sheet has properties approaching those of a homogeneous film or sheet of the binder polymer.

Color may be imparted to the sheet material of this invention by incorporating dyes or pigments in the polymeric binder, or by dyeing after finishing or using pre-dyed or pre-pigmented structural fibers. Preferably, colored sheet material is prepared by the use of dyed or pigmented structural fibers or by incorporating the coloring mat in the polymeric binder, since the sheet material is then uniformly colored throughout; and, thus, unlike colored natural leather, it will not exhibit any marked or undesirable color change if scuffed or abraded. When pigments are incorporated into the polymer binder for the purpose of preparing colored sheets, the concentration of pigments should be kept at a minimum, less than 5-10%, by weight of the total sheet, in order that the physical properties of the sheet, particularly tensile

strength, tear strength and abrasion resistance are not materially affected.

In following the process of the present invention, the creation of interconnecting pores or voids in the final sheet may be enhanced by distributing pore-forming fibers throughout the entire cross-section of the sheet. Consequently, interconnecting voids are then formed by extraction of pore-forming fibers and by stretching the sheet and/or by swelling-deswelling the sheet, this being highly useful when it is desired to form a leather replacement by combining a particular binder polymer with a particular fiber which adhere to each other to a degree greater than that normally practical when stretching and/or swelling-deswelling is used as the only means of imparting porosity to a particular fiber/binder sheet. On the other hand, it must be repeated that the greatest advantage of the present process is with respect to forming porous fiber-reinforced polymer sheets exhibiting an outstanding resistance to surface fuzzing upon scuffing by virtue of their having substantially no structural fibers or particles in the surface stratum.

The following examples will serve to further illustrate the nature of and techniques of preparing the leather replacement compositions of the present invention. Parts are by weight unless otherwise indicated.

#### EXAMPLE 1

A lay-up or composite was formed from three mats (1.8 oz./sq. yard) of non-woven fibers of polyhexamethylene adipamide, 2.5 inches in length and 3 denier per filament, and three homogeneous sheets or films (0.005"-0.006" in thickness) of a 50:50 blend of polyethylene and polyisobutylene as binder, alternately disposed with a fiber mat lowermost, and a top layer consisting of a mat of non-woven cellulose acetate fibers 2 inches in length and 3 denier per filament. This composite was subjected to a hot-pressing (step 1 of Figure 1) at a temperature of 140° C. at 500 p. s. i. for three minutes. The resulting compacted, substantially impermeable sheet took the form of stage B of Figure 1. Step 2 involved stretching the sheet of stage B in one direction to an extent substantially equal to 40% elongation. The resulting sheet was then in the form of stage C; that is, it was a porous fiber-reinforced sheet having soluble pore-forming fibers in the surface stratum. Finally, step 3 was effected; and this involved soaking the sheet in cold (room temperature) acetone to extract the soluble cellulose acetate fibers. The acetone exerted no solvent effect upon the nylon structural fibers and polyethylene-polyisobutylene binder. The leather permeability of the resulting sheet, stage D (0.020" in thickness), was within the range from 2,500-4,500 grams/100 sq. meters/hour. Furthermore, the composition was subjected to 20,000 scuffs before any fuzz appeared at the surface. This is in contrast with 50 scuffs, which pro-

ment comprising two wheels. One wheel was non-rotatable and was 6 inches in diameter and 1 inch in width. On the periphery of this wheel was mounted a sample of the sheet to be tested. The second wheel was made of felt, and it was 4 inches in diameter and 1 inch in width. The felt wheel rotated about an off-center axis (resulting in an eccentric motion), and the axis was so positioned that at the maximum displacement of the felt wheel, it abraded strongly against the sheet sample mounted on the larger non-rotatable wheel. A single rotation of the off-center wheel was referred to as a scuff.

#### EXAMPLES 2-5, INCLUSIVE

In the following examples, 2-5 inclusive, the binder polymer was incorporated into the initial composite in the form of films (0.002" in thickness) of polyethylene. The structural fibers were carded webs (weighing about 11 grams/sq. foot) of non-woven polyhexamethylene adipamide fibers (2½" in length and 3 denier per filament). The pore-forming or soluble fibers were in the form of mats (weighing about 5.5 grams/sq. foot) of non-woven cellulose acetate fibers (2" in length and 3 denier per filament). The initial lay-up was composed of alternate layers of webs of structural fibers and films of polyethylene, the bottom layer being a web of fibers and the uppermost binder layer being a homogeneous film of polyethylene. The web of cellulose acetate fibers was then placed upon the uppermost layer of polyethylene. Thereafter, the composite was subjected to heat and pressure in accordance with the conditions recorded in Table I below. The compacted composite sheet, which was substantially impermeable, i. e., non-porous, was then subjected to either a stretching step, that is, a stretch in two directions (30% by 40%), or the compacted sheet was immersed into a liquid which swelled the structural and pore-forming fibers, the liquid being at a temperature above the softening temperature of the binder polymer. (The liquid employed for swelling the structural fibers may also act as a solvent for the pore-forming fibers, or the pore-forming fibers may be extracted from the composition as a separate step.) After swelling the structural fibers at a temperature above the softening temperature of the binder polymer, the sheet was dried at a temperature approximately equal to the softening temperature of the binder polymer or at a lower temperature.

Table I indicates the thickness of the porous sheet, the unit weight of the sheet in grams per square meter, the leather permeability value (LPV), the temperature, pressure and time of pressing the initial composite, the extent to which the compacted sheet was stretched in both directions (when the sheet was stretched), and the time and medium in which the compacted sheet was immersed to swell the fibers. All of the sheets subsequent to stretching or swelling-deswelling were extracted in acetone for ten minutes to extract the pore-forming fibers.

Table I

| Example | Thickness of Final Sheet (inches) | Unit Weight of Final Sheet (gms./sq. meters) | LPV (gms./100 sq. meters/hour) | Pressed (°C., p.s.i. min.) | Stretched, percent | Swelled                         |
|---------|-----------------------------------|----------------------------------------------|--------------------------------|----------------------------|--------------------|---------------------------------|
| 2       | 0.05380                           | 902                                          | 2,1-9, 1, 867                  | 140°/500/6                 | 30 x 40            | 15 minutes in H <sub>2</sub> O. |
| 3       | 0.04113                           | 796                                          | 3, 681, 3, 245                 | 140°/350/6                 | -----              | 18 minutes in H <sub>2</sub> O. |
| 4       | -----                             | -----                                        | 2, 632, 2, 392                 | 140°/350/6                 | -----              | 22 minutes in H <sub>2</sub> O. |
| 5       | -----                             | -----                                        | 2, 355, 2, 276                 | 140°/350/6                 | -----              | -----                           |

#### EXAMPLES 6-9, INCLUSIVE

In the following examples, 6-9 inclusive, the binder polymer was in the form of films (0.003-0.004" in thickness) of a blend of polyethylene and polyisobutylene (50:50) or polyethylene alone. The structural fibers were in the form of carded webs (each weighing about 11 grams/sq. foot) of polyhexamethylene adipamide (2½" in length and 3 denier per filament). The pore-forming

duced fuzz at the surface of a similar composition which was prepared by stretching a structural fiber-reinforced polymeric sheet of the same composition, this sheet having structural fibers throughout its entire cross-section.

The scuff or abrasion resistance, i. e., resistance to surface fuzzing upon repeated abrasions, referred to in the foregoing example, was determined in a simple test instru-

fibers were either cellulose acetate or polyvinyl alcohol (in the form of non-woven mats weighing about 5.5 grams/sq. foot), the particular pore-forming fiber used being indicated in Table II below.

The binder polymer was formed into a film by casting the film from a hot solution of the polymers in toluene. A solution of polyisobutylene in toluene was effected at room temperature; the solution was heated; and polyethylene was added to the hot solution. The solution was then cast onto a smooth surface; and at the time when the film began to solidify, upon evaporation of the solvent, fibers of polyhexamethylene adipamide in the form of a mat were lightly pressed into the surface. The lay-up for Example 6 consisted of four layers of the binder polymer film, upon which were placed two layers (mats) of the structural fibers, four more layers of the binder polymer film, and, finally, a mat of pore-forming fibers, in the order named. The lay-ups for Examples 7 and 8 consisted of four mats of structural fibers alternated with four sheets of binder polymer film and a top mat of the pore-forming fiber. The lay-up for Example 9 consisted of two layers (mats) of the structural fibers on which were placed four films of the binder polymer, two more mats of structural fibers, four more films of the binder polymer, and a mat of the pore-forming fibers, in the order named. The web of pore-forming fibers was placed upon the uppermost layer of binder, and the composite was hot-pressed to form a consolidated structure. All of the composites were pressed at 140° C. and 500 lbs./sq. inch for 3 minutes. Table II indicates the thickness of the porous sheet, the unit weight in grams per square meter, the leather permeability, the extent to which the compacted sheet was stretched in both directions or the time during which the sheet was immersed in hot water (maintained at a temperature above the softening temperature of the binder polymer). In Example 9, the blend of polyethylene and polyisobutylene was employed as the binder polymer throughout the structure except at the uppermost surface of the sheet. For example, films of the upper four layers of binder polymer were polyethylene instead of a film of a blend of polyethylene and polyisobutylene. This provided for a flexible internal structure which, in turn, produced a final sheet having good flexibility, in addition to a surface layer having superior hardness and resistance to destruction on abrasion. Hence, by employing a surface film of the binder polymer which is different from the binder polymer employed internally, an integral structure may be formed, that is, as a result of hot-pressing the initial composite; but the surface of the final sheet may be improved by employing a binder polymer having greater toughness, hardness and resistance to abrasion than the binder polymer employed internally. It should be emphasized, however, that the binder employed in areas other than the surface of the sheet should be flexible and tough. As a general prerequisite in selecting a binder for use at the surface of a sheet, the binder polymer employed at the surface should exhibit good adhesion to the binder polymer employed internally in the sheet.

## EXAMPLE 10

In this example, the porous sheet was composed of the same binder polymer, structural fibers, and pore-forming fibers as those products of Examples 6-8, inclusive. Furthermore, the porous sheet was formed by stretching the initial compacted sheet 30% in both directions; and the pore-forming fibers (cellulose acetate) were extracted by immersing the sheet in acetone. Table III lists a number of physical properties of the porous sheet as compared with a range of the same properties of genuine leather.

## EXAMPLE 11

In this example, the binder polymer was in the form of a film cast from a solution of polyvinyl chloride and dioctyl phthalate (about 60%:40%) in methyl-ethyl ketone. The structural fibers were polyhexamethylene adipamide (2½" in length and 3 denier/filament); and the pore-forming fibers in the surface strata of the compacted sheet were polyvinyl alcohol fibers (2" in length and 3 denier/filament). The initial lay-up of components was similar to that illustrated by stage A of Figure 1, and the fiber mats of polyhexamethylene adipamide were lightly pressed into the cast films prior to complete evaporation of solvent. A fiber mat of polyvinyl alcohol fibers was placed upon the uppermost layer of binder polymer. The composite was pressed at 170° C. under a pressure of 350 lbs./sq. inch for 10 minutes and thereafter cooled below 100° C. under pressure. Table III indicates the extent to which the compacted sheet was stretched in both directions (30% by 30%), and the pore-forming fibers (polyvinyl alcohol) were extracted from the surface strata by immersing the stretched sheet in hot water. The physical properties of the final dried sheet are listed in Table III, and these properties are compared with range of the same properties of genuine leather compositions.

Table III

| 40                            | Physical Property | Leather Range | Example | Example |
|-------------------------------|-------------------|---------------|---------|---------|
|                               |                   |               | 10      | 11      |
| Thickness, inches             | .026-072          | 0.063         | 0.054   |         |
| Unit Weight, gms./sq. meter   | 567-1617          | 760           | 777     |         |
| Modulus, p. s. i.             | 1,000-15,000      | 4,200         | 12,153  |         |
| Percent Elongation to Break   | 35-112            | 110           | 94      |         |
| Tenacity, p. s. i.            | 1,725-6,200       | 3,279         | 4,927   |         |
| LPV, gms./100 sq. meters/hour | 220-13,000        | 3,419         | 4,937   |         |
| Scuff-felt Wheel Cycles       | 10,000            | 122,000       | 100,000 |         |
| Stretch, Percent              | 30 x 30           | 40 x 40       |         |         |
| Binder, Percent               |                   | 42            | 50      |         |

50

## EXAMPLE 12

An aqueous dispersion of neoprene was prepared, and the composition contained the following components:

- 55 1500 parts of neoprene latex.  
 96 parts of a commercial vulcanizing dispersion.  
 60 parts zinc oxide.  
 11 parts of a dispersing agent.  
 200 parts of a black pigment.

Table II

| Example | Thickness of The Final Sheet (inches) | Unit Weight of The Final Sheet (gms./sq. meters) | LPV          | Stretch/Swell |           | Pore-Forming Fiber | Extraction               | Binder                                                               |
|---------|---------------------------------------|--------------------------------------------------|--------------|---------------|-----------|--------------------|--------------------------|----------------------------------------------------------------------|
|         |                                       |                                                  |              | (Percent)     | (Minutes) |                    |                          |                                                                      |
| 6       | 0.04912                               | 803                                              | 2,745, 2,252 | 30 x 30       |           | Cellulose Acetate  | Acetone, 10 minutes      | Polyethylene/Polyisobutylene, 50/50                                  |
| 7       | 0.05550                               |                                                  | 8,298        | 30 x 30       |           | do                 | do                       | Do                                                                   |
| 8       | 0.05510                               |                                                  | 4,375        |               | 25        | Polyvinyl Alcohol  | Boiling H <sub>2</sub> O | Do                                                                   |
| 9       | 0.04266                               | 756                                              | 3,289, 2,570 | 30 x 30       |           | Cellulose Acetate  | Acetone, 15 minutes      | Polyethylene/Polyisobutylene (50/50); Polyethylene as surface binder |

## 19

The neoprene latex impregnating composition was prepared by adding the vulcanizing dispersion and zinc oxide to the neoprene latex, and thereafter mixing in a blend of the dispersing agent in water. This was mixed for about five minutes, and thereafter the black pigment was added and mixing was carried out for one hour. The dispersing agent and black pigment were dissolved in 650 parts of water.

Twelve non-woven mats of polyhexamethylene adipamide fibers (2½" in length and 3 denier/filament) were composited and sprayed on both surfaces with the neoprene latex composition, and the surface of the composite was sprayed with an additional quantity (about 4.9 parts by weight of the total composition). Before spraying the top web with additional latex, the weight ratio of binder polymer (neoprene) to fibers was about 60:40. On the top layer was placed a non-woven mat of fibers of polyvinyl alcohol (2" in length and 3 denier/filament). The resulting composite was consolidated at a temperature of 180° C. and 1,250 p. s. i. pressure for 10 minutes. Subsequently, the consolidated sheet was stretched 40% in both directions, and thereafter the soluble polyvinyl alcohol fibers in the upper surface stratum were extracted by immersing the sheet in hot water for 10 minutes. The resulting sheet was porous, and the surface stratum contained no structural fibers. The average LPV of several samples of this composition was in the neighborhood of 1,800 grams/100 sq. meters/hour, and the sheet was 0.0447" in thickness. The fiber-free surface was capable of being abraded or scuffed with an ink eraser without fuzzing.

## EXAMPLE 13

A terpolymer of beta-methoxyethyl acrylate/omega-chloroethoxyethyl acrylate/acrylic acid was cast from a solvent solution upon a film of a plasticized polyvinyl chloride. This binder combination served as the top binder layer in a composite comprising alternate layers of polyvinyl chloride binder and non-woven fibers of polyhexamethylene adipamide (2½" in length and 3 denier/filament). The top binder layer was the polyvinyl chloride film coated with the above terpolymer. The next layer beneath was a non-woven mat of the nylon fibers; the layer under that was a polyvinyl chloride film; and thereafter three more mats of fibers and two more films of polyvinyl chloride were superimposed. As the topmost layer, a web of polyvinyl alcohol fibers was placed upon the coated polyvinyl chloride binder. The relative weights of the components were as follows: 9.26 parts of nylon fibers, 9.68 parts of polyvinyl chloride binder, 1.98 parts of the terpolymer and 1.10 parts of the polyvinyl alcohol fibers.

The composite was consolidated by pressing at 170° C. under a pressure of 350 p. s. i. for 15 minutes. The resulting consolidated sheet was stretched 40% in both directions and thereafter placed in boiling water for 20 minutes to extract the polyvinyl alcohol pore-forming fibers from the surface stratum.

## EXAMPLE 14

Four individual mats of non-woven nylon fibers (polyhexamethylene-adipamide, 2½" in length and 3 denier/filament) were impregnated with the following neoprene latex and composited. The impregnating composition was composed of the following:

|                                                                                      | Parts |
|--------------------------------------------------------------------------------------|-------|
| Neoprene latex                                                                       | 820   |
| Plasticizer (oil-soluble sulfonic acid of high molecular weight with a paraffin oil) | 59    |
| Commercial dispersing agent                                                          | 53    |
| Sodium silicate                                                                      | 10    |

The weight ratio of binder polymer to fibers in this composition was approximately 60:40. The binder polymer was solidified by immersing the impregnated composite in

## 20

a 50:50 solution of acetic acid and methanol, followed by washing in water and drying at room temperature.

The upper surface of the impregnated composition was brushed with a black paint comprising chlorosulfonated polyethylene, and the coating was permitted to dry. On top of the coating were placed two layers of non-woven fibrous mats of polyvinyl alcohol fibers, and the composite was pressed at 140° C. and 500 p. s. i. for 15 minutes. The resulting consolidated sheet was stretched 40% in two directions, and the polyvinyl alcohol fibers were extracted in hot water. The resulting sheet had a leather-like surface texture, was permeable to water vapor, and resisted fuzzing upon being scuffed.

## EXAMPLE 15

Three composited individual layers of nylon non-woven fibers (polyhexamethylene adipamide, 2½" in length and 3 denier/filament) were impregnated with a plasticized polyvinyl chloride contained in solution in tetrahydrofuran, and the solvent was permitted to evaporate. A single layer of non-woven fibers of polyvinyl alcohol (2" in length and 3 denier/filament) was similarly impregnated with a plasticized polyvinyl chloride contained in solution using tetrahydrofuran as the solvent. The individually impregnated mats were composited so that the polyvinyl alcohol fibers were contained in the top layer, and the composite was consolidated by pressing at 140° C. and 500 p. s. i. for 10 minutes. The consolidated sheet was cooled under pressure and thereafter stretched 30% in two directions. The stretched sheet was then immersed in boiling water for one hour to extract the polyvinyl alcohol pore-forming fibers, and the sheet was dried. The parts by weight of the individual components in the consolidated sheet were as follows: 15.43 parts of nylon fibers, 16.27 parts of polyvinyl chloride binder, and 1.94 parts of polyvinyl alcohol pore-forming fibers. The resulting sheet was permeable to water vapor, and the surface containing no structural fibers was capable of being subjected to 100,000 scuffs before appreciable surface fuzzing was apparent.

## EXAMPLE 16

Individual carded non-woven webs of polyhexamethylene adipamide fibers (the web weighing approximately 2 ounces per square yard and the fibers being 1½" in length and 3 denier/filament) were individually impregnated by spraying one side of each web with the following composition:

|                     | Parts      |
|---------------------|------------|
| Polyvinyl chloride  | 50         |
| Diethyl phthalate   | 35         |
| Dimethyl sebacate   | 15         |
| Brown dye mixture   | 0.5-0.6    |
| Methyl ethyl ketone | about 2000 |

The sprayed webs were then dried at 50°-60° C. The degree of impregnation was regulated so that the binder polymer, that is, the polyvinyl chloride, constituted from 45-51%, by weight of the total weight of the impregnated webs.

Four of the impregnated webs were composited so that the "grains" (direction in which the webs were carded) were perpendicular to adjacent layers. The composite of webs was pressed at 125° C. and 500 p. s. i. for five minutes.

A topcoating (3 parts by weight per 81" of surface area) was then applied to the composited sheet structure, the top coating being sprayed as before, and the composition being the same as given above. A non-woven web of polyvinyl alcohol fibers (about 4.5 parts by weight per 81" of surface area) was laid upon the top coated surface of the consolidated sheet, and the composite was then pressed again at 120° C. and 500 p. s. i. for five minutes.

The composite film was then stretched 10% in two directions, and thereafter the polyvinyl alcohol fibers were extracted from the surface stratum by immersing the

structure between screens into a bath of boiling water for a period within the range from 2-10 minutes. After drying, the film was stretched further to an extent of 40% in both directions to form a porous leather replacement sheet, having a top surface which resisted surface fuzzing upon abrasion. The resulting sheet composition was permeable to air and water vapor.

I claim:

1. The process of forming non-woven, porous leather replacement fabrics which comprises associating substantially water vapor-impermeable, relatively extensible, initially thermoplastic, elastomeric, polymeric binder material with a fibrous sheet comprising essentially a non-woven base stratum of uniformly dispersed structural fibers of relatively non-extensible material, and a non-woven surface stratum of uniformly dispersed soluble pore-forming fibers and free of structural fibers to form an initial sheet, said pore-forming fibers being soluble in a solvent which is a non-solvent for the structural fibers, said binder material having a softening temperature below the softening temperature of said fibers; hot-pressing said initial sheet at a temperature above the softening temperature of said binder and below the softening temperature of said fibers, whereby to form a compacted substantially water vapor-impermeable sheet wherein said fibers are embedded in said binder; stretching said compacted sheet 10% to 50% in at least one direction to form channels substantially contiguous with the structural fibers distributed uniformly throughout the base stratum; and dissolving out said pore-forming fibers with a liquid which is a solvent for said pore-forming fibers and a non-solvent for said structural fibers and said binder material, whereby to form a porous, water vapor-permeable sheet of polymeric binder material reinforced with structural fibers and having a porous surface stratum free of fibers.

2. The process of claim 1 wherein the weight ratio of binder to structural fiber is within the range of from 30:70 to 70:30.

3. The process of claim 2 wherein the weight of said pore-forming fibers is within the range of from 5% to 25% of the total weight of fibers in said sheet.

4. The process of forming non-woven, porous, leather replacement fabrics which comprises associating initially thermoplastic, elastomeric, polymeric binder material with a fibrous sheet comprising essentially a non-woven base stratum of uniformly dispersed liquid-swellable structural fibers and a non-woven surface stratum of uniformly dispersed soluble pore-forming fibers free of structural fibers to form an initial sheet, said pore-forming fibers being soluble in a solvent which is a non-solvent for the structural fibers, said binder material having a softening temperature below the softening temperature of said fibers,

hot-pressing said initial sheet at a temperature above the softening temperature of said binder and below the softening temperature of said fibers whereby to form a compacted, substantially water vapor-impermeable, composite sheet wherein said fibers are embedded in said binder; soaking said compacted composite sheet at a temperature between the softening temperature of said binder and of said fibers in a liquid which swells the structural fibers; dissolving out said pore-forming fibers with a liquid which is a solvent for said pore-forming fibers and a non-solvent for said structural fibers and said binder material; and drying the resulting sheet at a temperature no greater than the softening temperature of the binder polymer to remove said liquid, whereby to form a porous, water vapor-permeable sheet reinforced with structural fibers and having a porous surface stratum free of fibers.

5. The process of claim 4 wherein the weight ratio of binder to structural fiber is within the range of from 30:70 to 70:30.

6. The process of claim 5 wherein the weight of said pore-forming fibers is within the range of from 5% to 25% of the total weight of fibers in said sheet.

7. A porous, water vapor-permeable leather replacement material comprising a sheet of initially thermoplastic, elastomeric, polymeric binder material having an integral porous surface stratum free of fibers; the remaining cross-section of the sheet being water vapor-permeable and having reinforcing structural fibers uniformly distributed throughout, the water vapor-permeability in said remaining cross-section being contributed solely by channels substantially contiguous with the structural fibers.

8. The product of claim 7 wherein the binder material of said surface stratum is different from the binder material of said remaining cross-section.

9. The product of claim 7 wherein the weight ratio of binder material to structural fibers is within the range of from 30:70 to 70:30.

10. The product of claim 7 wherein the weight of said binder material comprises from 40% to 60% of the total weight of binder and fibers.

11. The product of claim 7 wherein the structural fibers are at least 0.01 of an inch in length.

12. The product of claim 7 wherein the structural fibers are about 1.5 inches in length.

#### References Cited in the file of this patent

#### UNITED STATES PATENTS

|           |                |       |               |
|-----------|----------------|-------|---------------|
| 2,474,201 | Raymond et al. | ----- | June 21, 1949 |
| 2,650,184 | Biefeld        | ----- | Apr. 25, 1953 |
| 2,676,128 | Piccard        | ----- | Apr. 20, 1954 |